

No. 885,761.

PATENTED APR. 28, 1908.

E. F. KERN.

PROCESS OF RECOVERING METALS FROM THEIR SULFID ORES.

APPLICATION FILED SEPT. 1, 1906.



**Witnesses:**

William Campbell.  
E. L. Hurst.

**Inventor:**

Edward Frank Kern.

# UNITED STATES PATENT OFFICE.

EDWARD FRANK KERN, OF KNOXVILLE, TENNESSEE.

## PROCESS OF RECOVERING METALS FROM THEIR SULFID ORES.

No. 885,761.

Specification of Letters Patent.

Patented April 28, 1908.

Application filed September 1, 1906. Serial No. 333,018.

To all whom it may concern:

Be it known that I, EDWARD FRANK KERN, a citizen of the United States, residing at Knoxville, county of Knox, and State of Tennessee, have invented certain new and useful Improvements in Processes of Recovering Metals from their Sulfid Ores, of which the following is a specification, accompanied by drawing.

10 My invention relates to processes for the electrolytic recovery of metals from their sulfid ores by means of electrolysis, with the ore as anode in a fused electrolyte.

15 The principal object of my invention is to treat sulfid ores, and recovering therefrom the metals and the sulfur, with good metallurgical recovery, and at low cost.

20 Other objects will appear in connection with the following description of my method: I have discovered by experiment that if lead sulfid ore, which is a conductor of electricity, is made the anode in a suitable fused electrolyte, which has a melting point below that of the ore, the lead and associated metals of the 25 ore may be deposited at, or in, the cathode, while the sulfur, with which the metals are combined, is liberated from the bath, provided the temperature be above the boiling point of sulfur, which is 445° C. Frequently 30 the naturally occurring galena is too fine, being in the form of concentrates, or is associated with too much gangue material, to be directly suitable for the electrolysis; so I accordingly first melt the ore under a suitable 35 flux, thus collecting its metal content as a fused matte, which may be cast into suitable blocks or cylinders, and a slag, which contains most of the gangue material. Such blocks or cylinders of cast ore or matte, being 40 good conductors of electricity, are made the anodes, and also serve the purpose of carrying the current from an exterior conductor to the working surface of the anode. The cast 45 matte consists practically of the sulfids of lead, zinc, copper, iron, etc., and carries the gold, silver and other values of the ore.

50 As electrolytes, I prefer to use baths, containing lead chlorid. Fused lead chlorid has considerable dissolving power for lead sulfid, so the bath is nearly or quite saturated with lead sulfid, giving an electrolyte which is fluid at 500° C.

55 Other salts may be mixed with the lead chlorid, for example the haloid salts of the alkalies and alkaline-earths, and zinc chlorid.

I am not restricted to the use of chlorids

for the electrolyte, as the process will evidently succeed also with, for example, the fluorids, and mixtures of haloid salts with alkali hydroxids: the main object being to secure a bath which will melt at the proper temperature, not be too volatile, and conduct the current well.

60 Regarding the use of mixtures of salts, I have used:—2 parts NaCl + 1 part CaCl<sub>2</sub> + 1 part PbCl<sub>2</sub>; and 1 part NaCl + 2 parts CaCl<sub>2</sub> + 1 part PbCl<sub>2</sub>; and 3 parts NaCl + 1 part PbCl<sub>2</sub>. In all cases the mixtures were saturated, in their molten condition, with lead sulfid. These mixtures were fluid between 70 500° C. and 650° C.

65 The electrolysis, and the results, are similar with different suitable baths, or electrolytes; the main difference resulting from the different temperatures of working, which depend 75 upon the melting point of the bath, or electrolyte, used.

70 It is necessary that the melting point of the bath, or electrolyte, be below that of the sulfid ore, in order that the anode remains 80 solid. It is advantageous to use a bath, or electrolyte, which will melt and remain fluid in the region of 500° C., as a saving in the cost of keeping it molten is thus effected. A bath having a melting point below 450° C. 85 would be no great advantage, as a temperature of at least 50° above the boiling point of sulfur, which is 445° C., should be maintained in order to effect the rapid removal of the sulfur from the cell by volatilization. 90

95 The electric current efficiency, I have found in a number of experiments, to vary from 88% to 94%, the electromotive-force usually being about 2.5 volts with an anode current density of about 500 amperes per square foot. With a current density of about 1200 amperes per square foot, the electromotive-force varied from 4.5 to 6.0 volts. In either case, the distance from anode to cathode was from 1½ to 3 inches.

100 The lead which was reduced at the cathode was malleable, and free from sulfur, at least for all practical purposes, and the sulfur liberated at the anode was free from chlorin and sulfur chlorids.

105 I am enabled by my process to also recover the zinc occurring in lead ores. The zinc accumulates in the electrolyte, from which it may be recovered by any suitable method.

110 Having reference to the accompanying drawing, I have shown a view in vertical

cross-section of an apparatus in which I may carry out my invention. The apparatus consists of an iron vessel B, its inside walls lined with a refractory and non-conducting material D. This constitutes the electrolyzing cell, which contains the fused electrolyte E. The ore, or sulfid containing material, made into suitable form for electrolysis by fusing with a flux and the resulting matte 5 cast into blocks or a cylinder A, is placed in the electrolyte E, and brought into electrical contact with the (+) source of the current. The cathode C, is a bath of molten metal in the bottom of the cell B, which is in electrical 10 contact with the (-) source of the current. The molten metal cathode C, is maintained at a constant height by having a well G on the side of cell B, and as rapidly as the metal accumulates, it may be either ladled out or 15 else "tapped" from the apparatus. In order to recover the sulfur which is liberated at the anode during electrolysis, the apparatus may be provided with a cover H of refractory material, and the volatilized sulfur, or 20 its oxidized products, such as  $\text{SO}_2$ , removed 25 from the cell through the opening J.

The apparatus may be arranged above a suitable furnace F for the purpose of fusing the metal-cathode and the electrolyte, preparatory to the electrolysis, and for keeping the temperature constant during the operation.

What I claim as new and desire to secure by Letters Patent, is:

35 1. The process of recovering lead and associated metals from lead sulfid-containing ore which consists in treating the same to increase its electrical conductivity and then electrolyzing a suitable fused electrolyte comprising a metal haloid compound, with said treated material as anode.

2. The process of recovering lead and associated metals from lead sulfid-containing ore which consists in treating the same to increase 45 its conductivity and then electrolyzing a suitable fused electrolyte comprising a metal haloid compound and a metal sulfid, with said treated material as anode.

3. The process of recovering lead and associated metals from lead sulfid-containing ore which consists in fusing the same to remove 50 impurities and increase its electrical conductivity, and in electrolyzing a suitable fused electrolyte comprising a metal haloid compound, with said fused sulfid-containing material as anode.

4. The process of recovering lead and associated metals from lead sulfid-containing ore which consists in fusing the same to form a 55 matte and then electrolyzing a suitable fused electrolyte comprising a metal haloid compound and metal sulfid, with said matte as anode.

5. The process of recovering lead and associated metals from lead sulfid-containing ore

which consists in fusing the same to form a matte and then electrolyzing a suitable fused electrolyte comprising lead chlorid, with said matte as anode.

6. The process of recovering lead and associated metals from lead sulfid-containing ore which consists in fusing the same to form a matte and then in electrolyzing a suitable fused electrolyte comprising a metal chlorid and a metal sulfid, with said matte as anode. 70

7. The process of recovering lead and associated metals from lead sulfid-containing ore which consists in fusing the same to form a matte, and then in electrolyzing a suitable fused electrolyte comprising lead chlorid and 80 lead sulfid, with said matte as anode.

8. The process of recovering lead and associated metals from lead sulfid-containing ore which consists in fusing the same to form a matte, and then in electrolyzing a suitable 85 fused electrolyte comprising haloid compounds of lead and zinc having a metal sulfid dissolved therein, with said matte as anode.

9. The process of recovering lead and associated metals from lead sulfid-containing ore 90 which consists in fusing the same to form a matte, and then electrolyzing a suitable fused electrolyte comprising a haloid metal compound, at a temperature below the melting point of said material and above  $445^{\circ}\text{C}.$ , 95 with said matte as anode.

10. The process of recovering lead and associated metals from lead sulfid-containing ore which consists in fusing the same to form a matte, and then electrolyzing a suitable 100 fused electrolyte at a temperature of about  $500^{\circ}\text{C}.$ , said electrolyte comprising a metal haloid compound with said matte as anode.

11. A process of recovering lead and associated metals from lead sulfid-containing ore, 105 which consists in first fusing said ore with a suitable flux to form a matte and electrolyzing a suitable fused electrolyte, with the said matte as anode.

12. A process of recovering lead and associated metals from lead sulfid-containing ore, which consists in first fusing said ores with a suitable flux to form a matte and electrolyzing a suitable fused electrolyte, comprising a metal haloid compound, at a temperature below the melting point of the matte, with said matte as anode. 115

13. A process of recovering lead and associated metals from lead sulfid-containing ore, which consists in first fusing said ores with a suitable flux to form a matte and electrolyzing a suitable fused electrolyte, comprising a metal haloid compound, at a temperature above  $445^{\circ}\text{C}.$  and below the melting point of the matte with said matte as anode. 120

14. A process of recovering lead and associated metals from lead sulfid-containing ore, which consists in first fusing said ores with a suitable flux to form a matte and electrolyzing a suitable fused electrolyte, comprising a 125

130

haloid compound of lead and a haloid compound of an alkali or alkaline earth metal, at a temperature above 445° C. and below the melting point of the matte, with said matte 5 as anode.

15. A process of recovering lead and associated metals from lead sulfid-containing ore, which consists in first fusing said ores with a suitable flux to form a matte and electrolyzing 10 a suitable fused electrolyte, comprising haloid salts of lead, zinc and of an alkali or alkaline earth metal, at a temperature above 445° C. and below the melting point of the matte, with said matte as anode.

15. 16. A process of recovering lead and associated metals from lead sulfid-containing ore, which consists in first fusing said ore with a suitable flux to form a matte and electrolyzing 15 a suitable fused electrolyte, comprising

lead chlorid, at a temperature of about 500° 20 C., with said matte as anode.

17. A process of recovering lead and associated metals from lead sulfid-containing ore, which consists in first fusing said ores with a suitable flux to form a matte and electrolyzing 25 a suitable fused electrolyte, comprising lead chlorid, zinc chlorid and an alkali or alkaline earth haloid compound, having zinc sulfid dissolved therein, at a temperature of about 500° C., with said matte as anode.

In testimony whereof, I hereunto set my hand this thirtieth day of August 1906, in the presence of two subscribed witnesses.

EDWARD FRANK KERN.

Witnesses:

W.M. S. AUSTIN,  
R. B. SHERIDAN.